

Feb. 28, 1950

J. M. LAFFERTY

2,499,192

DISPENSER TYPE CATHODE

Filed Jan. 15, 1948

Fig.1.



Fig.2.

Fig.4.



Fig.5.



Fig.3.



Inventor:  
James M. Lafferty,

by *Merton D. Moore*  
His Attorney.

## UNITED STATES PATENT OFFICE

2,499,192

## DISPENSER TYPE CATHODE

James M. Lafferty, Schenectady, N. Y., assignor  
to General Electric Company, a corporation of  
New York

Application January 15, 1948, Serial No. 2,402

4 Claims. (Cl. 250—27.5)

1

My invention relates to dispenser type cathodes and methods of making the same.

Dispenser type cathodes have been manufactured in which a mesh of nickel or similar material is filled with a body of powdered electron emissive material such as barium aluminate. The mesh is heated by conduction current to raise the powdered material to a temperature at which electrons are emitted. For a number of applications, it is desirable to obtain a dispenser type cathode having relatively small cross sectional dimensions and it has been difficult to obtain satisfactory life from the cathode made in accordance with the prior art. Prior art dispenser cathodes have also possessed rather low resistance so that a relatively large heating current is required. In accordance with an important aspect of my invention, I provide an improved dispenser type cathode and an improved method of making it which results in a very dense supply of electron emitting material and as a result insures adequate emission for a long period of use.

It is an object of my invention to provide a new and improved dispenser type cathode.

It is another object of my invention to provide an improved dispenser type cathode which insures an adequate supply of electron emitting material over a long period of use.

It is another object of my invention to provide an improved dispenser type cathode and method of making which is particularly applicable to cathode structures of small cross sectional dimensions.

Further objects and advantages of my invention will become apparent as the following description proceeds, reference being had to the accompanying drawing, and its scope will be pointed out in the appended claims.

In the drawing, Fig. 1 is an end elevational view of a cathode assembly embodying my invention; Fig. 2 is a side elevational view of the cathode assembly shown in Fig. 1; Fig. 3 is a sectional view taken along the line 3—3 of Fig. 1; Fig. 4 is a perspective view of the cathode element of the assembly shown in Figs. 1-3; and Fig. 5 is a perspective view of apparatus which may be used to advantage in the manufacture of cathodes in accordance with my invention.

Referring now to the drawing, I have shown my invention as applied to a cathode assembly of a type which is particularly adapted for use in electron beam devices such as electron accelerators. As illustrated in the drawing, the cathode proper comprises a helical wire coil 1 which may be wound on a suitable mandrel and

2

have any desired cross section. As illustrated in Figs. 3 and 4, the cross section of the illustrated embodiment is rectangular. One side of the rectangle is curved inwardly or indented to provide focusing of the electron beam emitted from the cathode surface. The coil 1 is supported within a channel-shaped shield and focusing member 3 by means of an intermediate channel-shaped member including a central member 4 of molybdenum or similar material which is coated with a layer of alumina 5. As illustrated, the side walls of the channel member 3 extend beyond the curved surface of the cathode and adapt the shield for its focusing function. The cathode 1 and shield 3 may be supported in an electron discharge device, such as an electronic accelerator by the conductors 6 and 7 which may also provide means for supplying suitable potential to the shield 3. The ends 8 and 9 of the helical coil are brought out through openings in the channel 3 and are connected to suitable conductors 10 and 11 which are likewise sealed through the envelope of the device in which the cathode is to be used. The ends of the coil 1 are closed by sheet metal members 12 which are secured in position by welding or by the wires 13 which also bind the conductors 8 and 9 and 10 and 11 together. The cathode 1 and focusing shield 3 are positioned within a larger channel-shaped electrode 14 which extends beyond the inner shield 3 and may be utilized as an accelerating electrode. Suitable conductors 15 and 16 are bonded to the electrode 14 for supporting it within the device in which it is to be used in insulated relation with respect to the cathode assembly and permitting suitable positive voltage to be applied to it when it is to be used as an accelerating electrode.

In accordance with an important aspect of the present invention, the cavity provided by the helical wire coil 1 is filled with a dense body of electron emitting material designated by the numeral 17. While a number of materials may be used, such as barium hydroxide, thorium aluminate, or strontium aluminate, I have found that barium aluminate is particularly desirable. The barium aluminate in granular form may be loaded into the interior of the coil and the coil heated to a temperature of approximately 1650° C. (preferably in an atmosphere of hydrogen) to melt the barium aluminate. The barium aluminate forms a solid dense mass which only partially fills the interior of the coil 1 and the process is repeated until the coil is completely filled with a dense fused mass of solid barium aluminate. In the

completed cathode, the barium aluminate extends between adjacent turns of the coil sufficiently to insulate them with respect to one another and renders it possible for the coil 1 to function as a heater for the cathode. The coil offers appreciably higher resistance than the mesh employed in the dispenser cathodes of the prior art and the increased resistance reduces the heating current requirements of the cathode.

The method described above which involves alternately filling the coil with barium aluminate powder and melting it down works very satisfactorily and produces a cathode having a very dense solid core. I have found that it is possible to produce a cathode having essentially the same characteristics by melting a quantity of the barium aluminate and immersing the coil in the melted material. In Fig. 5, I have illustrated an electrically heated receptacle or boat which may be used for this purpose. As illustrated, the boat is shaped generally the same as the heater of the cathode to be filled with liquid barium aluminate and is formed of a suitable high temperature metal, such as molybdenum. The boat is provided with an electrical heating coil 19 which may be provided for melting the material. The cathode is immersed in the receptacle 18 which is substantially filled with melted barium aluminate. This is done preferably in an atmosphere of hydrogen or other reducing atmosphere. The heater and core are removed from the boat and after the assembly has cooled sufficiently the emitting material forms a solid dense core.

The cathode of my invention when employing barium aluminate is operated at temperatures of 1200-1350° C. which is sufficient to provide for the gradual release of barium from the supply provided by the dense core.

As an example of a cathode made in accordance with my invention, I have found that a coil of wire formed of 35 turns of .015 inch diameter wire provides a cathode approximately  $\frac{11}{16}$  of an inch long. This means that there is a very slight space between each turn which is filled with the solidified emissive material of the core. The dimension of the square coil may be, for example,  $\frac{1}{10}$  of an inch. A cathode having these dimensions and manufactured in accordance with my invention is capable of delivering a current of 500 milliamperes, and it has been found to have a useful life exceeding 10,000 hours. In the foregoing specification, two methods of produc-

ing the solidified core within the coil have been described. In both cases, the resultant mass may be considered as fused or cast and in the appended claims, the word "fused" is used to denote that the powdered material has been at least partially melted, that is, bonded together in a dense mass.

While I have shown and described a particular embodiment of my invention, it will be obvious to those skilled in the art that changes and modifications may be made without departing from my invention in its broader aspects, and I, therefore, aim in the appended claims to cover all such changes and modifications as fall within the true spirit and scope of my invention.

What I claim as new and desire to secure by Letters Patent of the United States is:

1. A cathode comprising a helical wire coil providing a heater and a cast body of electron emitting material within said coil and extending between adjacent turns of said coil to hold said turns in insulated relation.

2. A cathode comprising a helical coil of molybdenum wire and a cast mass of barium aluminate within said coil and extending between adjacent turns of said coil to hold said turns in insulated relation.

3. The method of making a dispenser type cathode which comprises forming a hollow coil and filling the coil with melted barium aluminate.

4. The method of making a cathode including a hollow supporting coil which comprises the steps of loading the coil with a quantity of emitting material in granular form, melting the material to form a dense mass and repeating the loading and melting steps until the coil is filled with a dense cast body of emitting material.

JAMES M. LAFFERTY.

#### REFERENCES CITED

The following references are of record in the file of this patent:

#### UNITED STATES PATENTS

| 45 | Number    | Name           | Date          |
|----|-----------|----------------|---------------|
|    | 1,813,704 | Lederer        | July 7, 1931  |
|    | 1,817,636 | Meyer et al.   | Aug. 4, 1931  |
|    | 1,946,603 | Von Wedel      | Feb. 13, 1934 |
| 50 | 2,007,926 | Braselton      | July 9, 1935  |
|    | 2,007,932 | Ruben          | July 9, 1935  |
|    | 2,107,945 | Hull et al.    | Feb. 8, 1938  |
|    | 2,175,345 | Gaidies et al. | Oct. 10, 1939 |